

Nov. 6, 1928.

1,690,253

J. SCHUMACHER

REINFORCED EDGE PLASTER BOARD

Filed Oct. 12, 1925

*Fig. 1*



*Fig. 2*



INVENTOR.

John Schumacher  
BY Nestall and Wallace  
ATTORNEYS.

## UNITED STATES PATENT OFFICE.

JOHN SCHUMACHER, OF LOS ANGELES, CALIFORNIA.

## REINFORCED-EDGE PLASTER BOARD.

Application filed October 12, 1925. Serial No. 61,981.

This invention relates to a plaster board formed with a cementitious core and having cover sheets of pliable material. It appertains more particularly to a board having its edge corners reenforced with resilient yielding material. The core of plaster board being of a substantially brittle cementitious material is frequently cracked, crushed, chipped, and otherwise injured at its corner edges during handling of the board. It also happens that the cover sheets are peeled back at the corners due to careless handling of the board.

The primary object of this invention is the provision of a plaster board having smooth reenforced corners at the edge, the latter being arranged to provide yielding resilient corners lending themselves to nailing to better advantage, less liable to injury and re-enforcing the board.

These objects together with other objects and corresponding accomplishments are obtained by means of the embodiment of my invention illustrated in the accompanying drawing, in which:

Fig. 1 is a perspective view showing a fragment of a plaster board panel at the edge, with a portion cut away to show a method of reenforcement; and Fig. 2 is a similar view showing another method of reenforcing the board.

Referring more particularly to Fig. 1, the usual plaster core 3 covered on its upper and lower faces with paper sheets 4 and 5 bonded to the core in the manner well known in the art is illustrated. The cover sheets are of such width that they may be turned under and embedded in the core as indicated by 6 and 7. These sheets are folded to provide a beaded corner, and enveloped in the corners and extending the length of the board are lengths of cord or twine indicated by 8 and 9. This construction provides a board which has smooth rounded corners of sufficient resiliency to act as yielding buffers and protect the plaster core. The embedded ends 6 and 7 act to reinforce the core at the edges, and the exposed edge face 10 is such that the cement putty used between panels will effectively adhere and bond itself to the board. It is obvious that all the edges or any number thereof may be reinforced in the manner described.

Referring more particularly to Fig. 2, the plaster core of a panel is indicated by 11

and the usual cover sheets by 12 and 13. The width of the cover sheets is greater than the plaster core, and in the formation of the core, the edges of the sheets are folded back upon themselves as indicated by 14 and 15. The folded edges are then bent at right angles to form overhanging corners or angles 16 and 17 leaving a partially exposed face 18. In this manner a protected corner having buffer qualities is provided, and at the same time, the raw edge of the cover sheets is embedded in the plaster core.

What I claim is:

1. A product of the character described comprising a cementitious core, a cover sheet of pliable material underfolded at the edge corner, the creased portion being beaded to form an edge corner and corner guard, and the cementitious core being exposed at the edge.

2. A product of the character described comprising a cementitious core, a cover sheet of pliable material underfolded at the edge corner, the inturned edge being embedded in the cementitious core and the creased portion being beaded to form an edge corner and corner guard.

3. A product of the character described comprising a cementitious core, a cover sheet of pliable material underfolded at the edge corner, the inturned edge being embedded in the plaster core and beaded to form an edge corner and corner guard, the cementitious core being exposed at the edge.

4. A product of the character described comprising a cementitious core, a cover sheet of pliable material underfolded at the edge corner, a length of cord enveloped in the creased portion to form with said cover sheets a bead forming an edge corner and providing a corner guard.

5. A product of the character described comprising a cementitious core, a cover sheet of pliable material underfolded at the edge corner, the inturned edge being embedded in the cementitious core, the creased portion at the edge being beaded to form an edge corner and corner guard, and a length of twine enveloped in the beaded portion.

6. A product of the character described comprising a cementitious core, a cover sheet of pliable material underfolded at the edge corner, the underfolded portion being embedded in the cementitious core at an angle to the remainder of the sheet, the corner

60

65

75

80

85

90

95

100

105

110

portion of the sheet formed by said fold being beaded to form a corner guard, a length of twine being encircled by the bead portion.

7. A product of the character described comprising a cementitious core, a cover sheet of pliable material underfolded at one edge, the folding line being beaded to form a cor-

ner guard and to project into the cementitious core to reenforce the corner.

In witness that I claim the foregoing I <sup>10</sup> have hereunto subscribed my name this 28th day of September, 1925.

JOHN SCHUMACHER.